

Oct. 1, 1968

M. N. ORNITZ ET AL

3,403,998

HIGH TEMPERATURE ALLOYS

Filed Feb. 5, 1965

Fig.1.



Fig.2.



Fig.3.



Fig.4.



Fig.5.



INVENTORS  
Martin N. Ornitz &  
Ray H. English

*Hooper, Leonard & Buel*  
*Their Attorneys*

1

3,403,998

## HIGH TEMPERATURE ALLOYS

Martin N. Ornitz, Wilkinsburg, and Ray H. English, McCandless Township, Allegheny County, Pa., assignors to Blaw-Knox Company, Pittsburgh, Pa., a corporation of Delaware

Filed Feb. 5, 1965, Ser. No. 430,544

3 Claims. (Cl. 75—171)

### ABSTRACT OF THE DISCLOSURE

A high temperature alloy having high strength resistance to corrosion and thermal shock and low creep at temperatures up to 2500° F. of the composition, up to 1% carbon, about 26 to 38% chromium, up to 0.2% manganese, up to 0.2% silicon, about 10% to 25% tungsten and the balance nickel with residual impurities in ordinary amounts.

This invention relates to high temperature alloys and more particularly to an alloy and parts made therefrom having high strength and low creep at temperatures up to 2500° F. coupled with resistance to corrosion and thermal shock. The need for alloys having high strength and low creep, coupled with resistance to corrosion and thermal shock in the temperature range of 2400° F., has long been recognized. Such alloys are particularly desirable instead of ceramic refractories and the like in roller-type furnaces and slab heaters as well as in radiant heat tubes and the like which are operated in the temperature range of 2400° F. Conventional alloys used for applications in this temperature range have not been satisfactory for most uses because of the high rate of creep, corrosion and lack of strength at temperatures at or about 2200° F. to 2500° F.

We have discovered an alloy composition having high strength and low creep characteristics coupled with corrosion resistance and high resistance to thermal shock at temperatures up to 2500° F. The surprising characteristics of this alloy appear to be particularly dependent upon the control of carbon, iron and tungsten within a critical nickel-chromium base analysis. The broad composition range of the alloy of this invention lies within the following limits:

|          |                                                    |
|----------|----------------------------------------------------|
| C -----  | Up to about 1.0%.                                  |
| Cr ----- | About 26% to about 38%.                            |
| W -----  | About 10% to about 25%.                            |
| Mn ----- | About 0.2% maximum.                                |
| Si ----- | About 0.2% maximum.                                |
| Ni ----- | Balance with usual impurities in ordinary amounts. |

The foregoing broad alloy composition will provide alloys which give generally satisfactory results at temperatures up to about 2500° F. We have found, however, that for continued service at or above 2100° F. the following narrower range of composition should be observed:

|          |                          |
|----------|--------------------------|
| C -----  | Percent (about) 0.2-0.75 |
| Cr ----- | 28-35                    |
| W -----  | 13-19                    |
| Ni ----- | 40-60                    |

A single preferred composition would be:

2

|   |    | Percent (about) |
|---|----|-----------------|
| 5 | C  | 0.5             |
|   | Cr | 31              |
|   | Ni | 51              |
|   | W  | 17              |

With balance impurities in ordinary amounts

We have found that the above ranges must be observed if the desired high strength, low creep corrosion resistance and resistance to thermal shock at the higher temperatures here contemplated are to be achieved. We have found that as the temperature of service increases, the carbon content should preferably be on the low end of the stated carbon range and that the manganese and silicon should be low as should the usual impurities associated with nickel, such as iron.

The unusual properties of our alloy and the criticality of the composition are perhaps best illustrated by comparison of the following test results and examples.

### Example I

A group of alloys were melted to evaluate the effectiveness of various combinations within the broad range of the invention in creep control at 2400° F. The alloys were formed and tested at 2400° F. in a standard cantilever creep test using 250 lb./in.<sup>2</sup> loading with the following results:

TABLE I

| 30      | Analysis, Percent |      |       |   | Rate of Creep, rad./hr. |
|---------|-------------------|------|-------|---|-------------------------|
|         | Ni                | Cr   | C     | W |                         |
| 48.2    | 37.1              | .02  | 9.95  |   | .00021                  |
| 49.0    | 31.7              | .02  | 14.44 |   | .00038                  |
| 45.0    | 34.3              | .02  | 13.77 |   | .00035                  |
| 47.7    | 33.7              | .27  | 14.38 |   | .00021                  |
| 48.5    | 33.0              | .41  | 14.11 |   | .00011                  |
| 48.4    | 33.3              | .52  | 14.52 |   | .0001                   |
| 48.1    | 33.7              | .67  | 14.76 |   | .00002                  |
| 48.0    | 33.5              | 1.01 | 14.20 |   | .00023                  |
| 47.8    | 33.3              | .59  | 14.35 |   | .0004                   |
| 47.5    | 29.1              | .59  | 18.75 |   | .00012                  |
| 47.7    | 24.2              | .61  | 24.16 |   | .00046                  |
| 47.3    | 19.2              | .56  | 29.67 |   | rapid                   |
| 35 51.5 | 28.7              | .57  | 14.82 |   | .0017                   |
| 57.4    | 24.5              | .61  | 14.17 |   | rapid                   |
| 46.8    | 29.5              | .01  | 19.4  |   | .00011                  |
| 47.7    | 29.8              | .31  | 17.2  |   | .00018                  |
| 48.4    | 30.0              | .01  | 19.92 |   | .0054                   |
| 48.8    | 30.5              | .04  | 18.8  |   | .0012                   |
| 47.7    | 30.8              | .10  | 19.4  |   | .0027                   |
| 49.6    | 30.4              | .15  | 19.12 |   | .00123                  |
| 45 47.9 | 30.3              | .19  | 20.2  |   | .00067                  |
| 48.5    | 30.7              | .31  | 18.8  |   | .0048                   |
| 48.2    | 29.9              | .37  | 19.4  |   | .00088                  |
| 59.1    | 29.9              | .38  | 9.12  |   | .0200                   |
| 55.5    | 29.7              | .37  | 13.6  |   | .0040                   |
| 52.8    | 28.9              | .40  | 14.8  |   | .0025                   |
| 50.7    | 28.6              | .41  | 17.36 |   | .0026                   |
| 50.0    | 30.1              | .40  | 19.76 |   | .0047                   |
| 47.4    | 29.6              | .40  | 20.96 |   | .0051                   |
| 45.7    | 29.0              | .40  | 22.72 |   | .0180                   |
| 53.5    | 31.8              | .05  | 14.7  |   | .00037                  |
| 55.1    | 30.6              | .04  | 15.4  |   | .0027                   |
| 52.7    | 30.8              | .03  | 16.4  |   | .0017                   |
| 53.0    | 31.1              | .05  | 17.6  |   | .0027                   |
| 50.0    | 30.7              | .01  | 17.3  |   | .00053                  |

This data is plotted in FIGURE 1.

### Example II

A series of alloys were melted at the 14% tungsten level with various carbon contents to determine the effect of carbon. The results are plotted in FIGURE 2.

### Example III

A series of alloys at 0.6% carbon and at 0.4% carbon with varying tungsten were made. The chromium content was 30% and the nickel varied with tungsten to produce a nickel and tungsten content of 70% in FIGURE 3. In

FIGURE 4 the nickel content was maintained at 48% and the chromium varied with tungsten to produce a chromium and tungsten content of 50%.

Example IV

Stress rupture data were determined on several alloys whose analyses were as follows:

TABLE 2(A)

| C   | Mn  | Si  | Ni   | Cr   | W    |
|-----|-----|-----|------|------|------|
| .01 | .02 | .06 | 47.5 | 30.7 | 20.0 |
| .05 | .01 | .06 | 49.5 | 30.6 | 19.8 |
| .01 | .01 | .07 | 50.0 | 28.6 | 20.0 |
| .01 | .01 | .02 | 49.8 | 28.2 | 20.0 |
| .01 | .02 | .18 | 47.7 | 30.7 | 19.8 |
| .38 | .02 | .02 | 48.5 | 29.5 | 20.0 |
| .66 | .02 | .10 | 46.1 | 27.3 | 20.5 |
| .48 | .02 | .04 | 32.3 | 49.0 | 16.4 |
| .23 | .01 | .01 | 44.6 | 31.7 | 19.0 |
| .38 | .02 | .02 | 48.5 | 29.5 | 20.0 |
| .31 | .01 | .01 | 45.8 | 31.6 | 19.0 |
| .41 | .01 | .01 | 45.8 | 31.7 | 19.0 |
| .10 | .01 | .01 | 45.8 | 31.6 | 19.0 |
| .55 | .01 | .01 | 50.5 | 29.7 | 19.0 |

The stress rupture data are set out in the following table:

TABLE 2(B)

| C        | Stress | Rate   | Time to Rupture |
|----------|--------|--------|-----------------|
| 2,400 F. |        |        |                 |
| .00      | 350    | .0019  | 153             |
| .05      | 350    | .025   | 18              |
| .00      | 350    | .001   | 158             |
| .00      | 400    | .0012  | 350             |
| .00      | 272    | .00065 | 1,520           |
| 2,300 F. |        |        |                 |
| -----    | 665    | .0127  | 184             |
| -----    | 1,000  | .0187  | 67              |
| -----    | 300    | .001   | 552             |
| .38      | 500    | .0003  | 663             |
| .66      | 660    | .00025 | 300             |
| .66      | 1,000  | .00025 | 76              |
| .48      | 500    | .013   | 496             |
| 2,200 F. |        |        |                 |
| .66      | 1,500  | .088   | 30              |
| .66      | 1,000  | .011   | 190             |
| .48      | 750    | .0002  | 1,830           |
| 2,100 F. |        |        |                 |
| .66      | 1,750  | .38    | 83              |
| 2,000 F. |        |        |                 |
| .66      | 3,000  | .052   | 125             |
| .66      | 2,500  | .0108  | 212             |
| .66      | 2,000  | .0096  | 595             |
| 1,950 F. |        |        |                 |
| .45      | 2,000  | .0019  | 1,870           |
| .35      | 2,000  | .0021  | 1,260           |
| .55      | 1,600  | .00028 | 1,681           |
| .23      | 1,600  | .0022  | 1,2378          |

1,850 F.

|   |     |       |       |       |
|---|-----|-------|-------|-------|
| 5 | .38 | 5,000 | .0092 | 350   |
|   | .35 | 4,000 | .0046 | 850   |
|   | .45 | 4,000 | .0044 | 825   |
|   | .10 | 4,000 | ----- | 330   |
|   | .55 | 3,000 | .0009 | 1,685 |

<sup>1</sup> No fracture.

The foregoing stress rupture characteristics are shown in FIGURE 5.

The foregoing tables and accompanying drawings clearly illustrate the criticality of the composition of this alloy and the very significantly improved creep resistant properties.

15 While we have described certain preferred embodiments of our invention in the foregoing specification, it will be understood that the invention may be otherwise embodied within the scope of the following claims.

We claim:

20 1. A low creep, high strength alloy resistant to corrosion and thermal shock at temperatures up to 2500° F. consisting essentially of an effective amount up to about 1.0% carbon to provide high strength, corrosion resistance and low creep at elevated temperatures, about 26% to 38% chromium, up to about 0.2% manganese, up to about 0.2% silicon, about 10% to 25% tungsten and the balance nickel with residual impurities in ordinary amounts.

30 2. A low creep, high strength alloy resistant to corrosion and thermal shock at temperatures up to 2500° F. consisting essentially of about 0.20% to 0.75% carbon, about 28% to 35% chromium, up to about 0.2% manganese, up to about 0.2% silicon, about 13% to 19% tungsten and the balance nickel with residual impurities in ordinary amounts.

35 3. A low creep, high strength alloy resistant to corrosion and thermal shock at temperatures up to 2500° F. consisting essentially of about 0.5% carbon, about 31% chromium, about 17% tungsten and the balance nickel with residual impurities in ordinary amounts.

40 4. A low creep, high strength alloy resistant to corrosion and thermal shock at temperatures up to 2500° F. consisting essentially of about 0.5% carbon, about 31% chromium, about 17% tungsten and the balance nickel with residual impurities in ordinary amounts.

References Cited

UNITED STATES PATENTS

|           |        |         |       |        |
|-----------|--------|---------|-------|--------|
| 1,774,862 | 9/1930 | Wissler | ----- | 75—171 |
| 2,396,552 | 3/1946 | Cape    | ----- | 75—171 |
| 2,458,502 | 1/1949 | Cape    | ----- | 75—171 |

RICHARD O. DEAN, Primary Examiner.

HYLAND BIZOT, Assistant Examiner.